

# United States Patent

[19]

Senez

[11] 3,765,831

[45] Oct. 16, 1973

[54] TREATMENT OF POLYPEPTIDE FIBRES

[75] Inventor: Claude Jean Michel Senez,  
Chantilly, France

[73] Assignee: Ugine Kuhlmann, Paris, France

[22] Filed: Nov. 2, 1971

[21] Appl. No.: 195,019

[30] Foreign Application Priority Data

Nov. 3, 1970 France 7039457

[52] U.S. Cl. 8/54, 8/86, 8/169,  
8/172, 8/173

[51] Int. Cl. D06p 3/14

[58] Field of Search 8/54, 86, 41 B, 42 B,  
8/173, 169

[56] References Cited

UNITED STATES PATENTS

3,334,960 8/1967 Abel 8/54  
3,104,931 9/1963 Casty et al. 8/54

3,218,116 11/1965 Casty et al. 8/54

Primary Examiner—Leon D. Rosdol

Assistant Examiner—T. J. Herbert, Jr.

Attorney—Francis C. Browne et al.

[57] ABSTRACT

The present invention provides a process for dyeing polypeptide fibres which comprises dyeing said fibres with an anionic dyestuff in the presence of (1) at least one polyoxyalkylenated non-ionic dispersing agent resulting from the condensation of an alkylene oxide with an aliphatic alcohol or an alkylphenol and (2) at least one polyoxyalkylenated condensate resulting from the condensation of an alkylene oxide with an aliphatic amine containing 12 to 20 carbon atoms and esterification with an oxygen-containing polyacid. There are also provided compositions comprising said dispersing agents and said polyoxyalkylenated condensates.

7 Claims, No Drawings

## TREATMENT OF POLYPEPTIDE FIBRES

The present invention relates to surface active compositions. It also relates to the use of such compositions in the dyeing of polypeptide fibres, especially wool, so as to obtain a rapid fixing of the dyestuffs without affecting the evenness of the shades. 5

It is known that dyeing of polypeptide fibres, especially wool, at boiling temperature, causes degradation of the fibrous substance and a modification of their properties. Operation at elevated temperature (98° to 100° C.), at a pH close to neutrality in order to ensure a proper evenness of shade, and operation for a sufficiently long time, leads to a loss of amino acids. A reduction of the tensile strength of the fibres thus treated results, as well as a reduction of their natural elasticity. The yarns or fabrics which have received this dyeing treatment lose a part of their good qualities such as brightness or fullness for which they are generally valued. In addition, this fairly long dyeing process is relatively tedious although the shades obtained have excellent fastness, for example to light, rubbing or washing, as well as an excellent tinctorial yield. 15

By means of the present invention the dyeing temperature can be appreciably lowered, the period of treatment can be reduced and the operation can be effected at a lower pH which is near to the isoelectric point of the material, while obtaining an excellent tinctorial yield as well as general fastness equivalent to that obtained by the prior technique. Lowering of the pH of the dyebath is not itself normally effected without difficulties, since a more acid pH considerably increases the affinity of the dyestuff for the fibres and this increase is not compensated by the lowering of the temperature. Lack of evenness was to be feared. Besides the advantageous results mentioned above, the process according to the present invention enables uniform shades to be obtained with a variety of anionic dyestuffs used for dyeing wool. These dyestuffs are characterised generally by the fact that they possess sulphonic or carboxylic groups and consequently may belong to the class of acid dyestuffs as defined in the Colour Index (Volume I, 1956, page 1,001) or to the class of the mordant dyestuffs (Colour Index, page 1,405). Among the latter, the dyestuffs described in U.S. Pat. specification No. 3,547,572 or British Pat. specification No. 1,001,182 may be particularly mentioned. The 1:2 metalliferous complexes may also be advantageously used in the process of the invention. 25

According to the present invention there is provided a process for dyeing polypeptide fibres which comprises dyeing said fibres in the presence of (1) at least one polyoxyalklenated non-ionic dispersing agent resulting from the condensation of an alkylene oxide with an aliphatic alcohol or an alkylphenol and (2) at least one polyoxyalklenated condensate resulting from the condensation of an alkylene oxide with an aliphatic amine containing 12 to 20 carbon atoms and esterification with an oxygen-containing polyacid. 35

The present invention also provides a composition comprising an aqueous mixture of (1) at least one polyoxyalklenated non-ionic dispersing agent resulting from the condensation of an alkylene oxide with an aliphatic alcohol or an alkylphenol and (2) at least one polyoxyalklenated condensate resulting from the condensation of an alkylene oxide with an aliphatic amine containing 12 to 20 carbon atoms and esterification with an oxygen-containing polyacid. 45

Esters of the above type (2) include those of the general formula:



wherein R represents a saturated or unsaturated aliphatic radical containing 12 to 20 carbon atoms, m and n each represents a whole number, the sum m+n being from three to 20, p represents one or two and X represents the residue  $\text{SO}_3\text{Y}$  or the residue  $\text{PO}_3\text{Y}_2$ , Y representing a hydrogen atom, an alkali metal, the ammonium group or the residue of an organic base of low molecular weight. Compounds of this type have been described, for example, in French Pat. specification No. 1,542,683 of Sept. 4, 1967. 15

The non-ionic dispersing agents of type (1) include those of the general formula:



wherein R' represents an aliphatic or alkylphenyl radical containing 10 to 22 carbon atoms and q is a whole number from 10 to 50, preferably from 15 to 25. Such compounds include, for example, the polyoxyethylenated derivatives of lauryl, myristyl, cetyl, or stearyl alcohols or of octyl, nonyl, decyl and dodecyl phenols. 20

The polyoxyalklenated non-ionic dispersing agents (1) and the polyoxyalklenated esters (2) are preferably used in such amounts that the ratio of the first to the second is between 0.6 and five (by weight). The use of more than one compound of each of types (1) and (2) is within the scope of the present invention. 25

The operation is advantageously carried out as follows: The polypeptide fibres are treated in the aqueous bath containing one or more compounds of each of type (1) and (2) at a pH near to the isoelectric point of the fibres, and at a temperature between 40° and 85° C., the dyestuff is added and dyeing is effected at an approximately constant temperature not exceeding 85° C. 30

The following Examples illustrate the invention without restricting it. The percentages are by weight unless otherwise specified. 35

## EXAMPLE 1

A dyebath is prepared containing 0.5 percent of the product obtained from the condensation of 50 moles of ethylene oxide with one mole of lauryl alcohol and 0.5 percent of the amphoteric derivative obtained by condensation of 10 moles of ethylene oxide with one mole of oleylamine followed by sulphation and neutralisation with soda, these amounts being calculated on the weight of the material to be dyed. The pH of the bath is adjusted to 5 by means of acetic acid and sodium acetate. 50

A woollen fabric is treated for 5 minutes in the bath at 40° C., the ratio of the material to be dyed to the volume of the bath being one to 40. 0.8 percent (based on the weight of wool) of the 1:2 chromium complex of 3',4'-dichloro-2'-hydroxy-4-phenylazo-1-p-sulphophenyl-3-methyl-5-hydroxy-pyrazole and of the 5'-chloro-2'-hydroxy-4-phenyl-azo-1-phenyl-3-methyl-5-hydroxy pyrazole are introduced, then the temperature is raised to 85° C. in a period of 40 minutes. This temperature is maintained for 40 minutes, and the fabric is rinsed and dried. 55

The red shade obtained is even and has a fastness comparable with that obtained by dyeing at 95° to 100° C. for 1 hour or 1½ hours at pH 6.

#### EXAMPLE 2

A dyebath is prepared containing 0.65 percent of the product obtained from the condensation of 20 moles of ethylene oxide with one mole of nonylphenol and 0.35 percent of the amphoteric derivative obtained by sulphation and neutralisation with ammonia of the product resulting from the condensation of 7 moles of ethylene oxide with one mole of laurylamine, these quantities being determined by weight with respect to the material to be dyed for a bath ratio of one to 12. The pH of the bath is adjusted to 5 by addition of acetic acid and sodium acetate and bobbins of woollen yarn are treated for 10 minutes at 85° C. by circulation of the bath. The following are then introduced at this temperature: 0.04 percent of the 1:2 chromium complex of 5'-chloro-2'-hydroxy-2-phenylazo-1-hydroxy-4-methyl-naphthalene and of 4'-sulpho-2'-hydroxy-1-phenylazo-2-hydroxy-naphthalene, 0.1 percent of the 1:2 chromium complex described in Example 1, 0.2 percent of the 1:2 chromium complex of 5'-nitro-2'-hydroxy-4-phenylazo-1-m-sulphophenyl-3-methyl-5-hydroxy-pyrazole and of 5'-nitro-2'-hydroxy-4-phenylazo-1-phenyl-3-methyl-5-hydroxy-pyrazole.

The temperature is maintained at 85° C. for an hour, the direction of circulation of the bath being changed every 5 minutes, then the yarn is rinsed and dried. The rose beige shade obtained is uniform and has the fastness which would be obtained by dyeing at 95° to 100° C. at pH 6.5.

#### EXAMPLE 3

A dyebath is prepared containing 1 percent of the product obtained from the condensation of 23 moles of ethylene oxide with one mole of stearyl alcohol and 0.4 percent of the amphoteric derivative described in Example 2, these quantities being calculated on the weight of the material to be dyed for a bath ratio of one to 15. The pH of the bath is adjusted to 5 by addition of acetic acid and sodium acetate. The wool, in the form of flock, is treated for 10 minutes at 85° C. by circulation of the bath. 1.2 percent of the 1:2 chromium complex of 3'-nitro-2'-hydroxy-2-phenylazo-5-sulpho-1-hydroxy-naphthalene and of 3'-nitro-2'-hydroxy-1-phenylazo-2-hydroxy-4-diethylamino-benzene is then introduced at this temperature.

This temperature of 85° C. is maintained for an hour, the direction of circulation of the bath being changed every 5 minutes. The wool is then rinsed and dried. The blue shade obtained is even and has excellent fastness.

#### EXAMPLE 4

A dyebath is prepared containing 0.9 percent of the product obtained from the condensation of 20 moles of ethylene oxide with 1 mole of oleyl alcohol and 0.3 percent of the amphoteric derivative obtained by phosphatization of the product resulting from the condensation of 6 moles of ethylene oxide with 1 mole of laurylamine and neutralisation with ammonia, these quantities being calculated on the weight of the material to be dyed. After adjusting the pH to 5, a woollen felt fabric is treated at 40° C. for 5 minutes in this bath, the bath ratio being 1 to 40. 0.5 percent (based on the weight of the fibres) of the 1:2 chromium complex of

5' -nitro-2'-hydroxy-4-phenylazo-1-m-sulphophenyl-3-methyl-5-hydroxy-pyrazole and of 5'-nitro-2'-hydroxy-4-phenylazo-1-phenyl-3-methyl-5-hydroxy-pyrazole is then introduced and the temperature is raised to 85° C. in a period of 40 minutes. It is maintained at this temperature for 40 minutes. The fabric is then rinsed and dried.

The orange shade obtained is uniform and has a fastness equivalent to that obtained by dyeing at 95° to 100° C. at pH 6.5.

#### EXAMPLE 5

A dyebath is provided containing 0.75 percent of the product obtained from the condensation of 20 moles of ethylene oxide with one mole of nonyl phenol and 0.25 percent of the amphoteric derivative obtained by sulphation followed by neutralisation with ammonia of the product resulting from the condensation of 7 moles of ethylene oxide with one mole of laurylamine, these quantities being calculated on the weight of the material to be dyed with the bath ratio being 1 to 12.5. The pH of the bath is buffered at 5 by addition of acetic acid and sodium acetate. Bobbins of woollen yarn are treated at 85° C. for 10 minutes by circulating the bath. 1 percent of the 1:2 naphthalene chromium complex described in Example 2 is then introduced at this temperature. The temperature is maintained at 85° C. for an hour, the direction of circulation of the bath being reversed every 5 minutes. The yarn is rinsed and dried. A perfectly uniform anthracite grey shade is obtained, the fastness of which is equivalent to that of a dyeing at the boil at pH 6.

#### EXAMPLE 6

35 A dyebath is prepared containing 0.55 percent of the product obtained from the condensation of 20 moles of ethylene oxide with 1 mole of nonylphenol and 0.30 percent of the amphoteric derivative obtained by bisulphation followed by neutralisation with ammonia of the product resulting from the condensation of 11 moles of ethylene oxide with one mole of copra amine ("Noramox C<sub>11</sub>"), these quantities being determined by weight with respect to the material to be dyed for a bath ratio of one to 12. The pH of the bath is adjusted to 4.5 by addition of acetic acid and sodium acetate. 2 G. per litre of ammonium sulphate are then added and the wool in the form of flock is treated for 5 minutes in the bath at 40° C. The following substances are introduced at this temperature:

40 1.8 percent of 2'-hydroxy-1'-naphthalyl-1-azo-4-sulpho-2-hydroxy-naphthol in dispersed state;  
45 0.3 percent of (2,6-dichloro)phenyl-(3-methyl-4-hydroxy-5-carboxy)-phenyl-(3-carboxy-4-oxo-5-methyl)-2,5-ylidene-cyclohexadiene-methane;  
50 0.3 percent of bis(3-carboxy-4-hydroxy-5-methyl-phenyl)-(3-carboxy-4-oxo-5-methyl)-2,5-ylidene-cyclohexadiene-methane.

The temperature is rapidly raised to 85° C. and is maintained at this figure for 40 minutes. At the same temperature 1.2 percent of sodium dichromate is then introduced and the temperature raised rapidly to 102° C. The temperature is maintained at 102° C. for 20 minutes, then the material is rinsed and dried. The blue shade obtained is uniform and has a fastness which is obtained on effecting the dyeing at pH 6 and at 95° to 100° C. for 1 hour to 1½ hours and chroming at 102° C. for one-half hour.

## EXAMPLE 7

A dyebath is prepared with the same quantities of products described in Example 6. The pH of the bath is adjusted to 5 by addition of acetic acid and sodium acetate. 2 G. per litre of ammonium sulphate are then added. Bobbins of woollen yarn are treated by circulation of the bath while rapidly raising the temperature from 40° to 60° C. Then the following are introduced at 60° C:

- 0.15 percent of [3,2'-dicarboxy-4-phenylaminosulphonyl-benzene]-<1 azo 5>-[1-methyl-3-phenyl-4-hydroxy-pyrazole] in a dispersed state;
- 0.18 percent of 4-(3-methyl-5-nitro-6-hydroxy)-phenylazo-1-(4-sulpho)-phenyl-3-methyl-5-hydroxy-pyrazole;
- 0.20 percent of 8-(2-hydroxy-3-chloro-4-sulpho)-phenylazo-1-acetalamino-7-naphthol.

The temperature is raised to 90° C. in a period of 50 minutes. 0.3 percent of sodium dichromate is then introduced and the temperature is raised to 102° C. This temperature is maintained for 15 minutes, then the material is rinsed and dried. The rose beige shade obtained is uniform and has a fastness equal to that obtained by dyeing at pH 6 according to the standard process at 95° to 100° C. which takes 2½ hours.

## EXAMPLE 8

A dyebath is prepared with the same quantities of the products described in Example 6. The pH of the bath is adjusted to 5. 2 G. per litre of ammonium sulphate and 10 percent of sodium sulphate, determined by weight with respect to the material to be dyed for a bath ratio of one to 40, are then added. Material consisting of wool-polyamide pullovers is treated for 20 minutes at 40° C. 1.5 percent of [3'-sulpho-4-phenylazo-naphthalene]-<1 azo 1>-[5-sulpho-4-phenylamino-naphthalene] is then introduced.

The temperature is maintained at 40° C. for 20 minutes and is then raised to 85° C. in a period of 40 minutes. It is maintained at this temperature for 45 minutes. The material is then rinsed and dried.

The blue shade obtained is uniform and the seams are perfectly penetrated. In addition, the fastness to water and to washing is comparable with that of a dyeing effected at the boil.

## EXAMPLE 9

A dyebath is prepared with half the quantities of the products described in Example 6. The pH of the bath is adjusted to 4.5 by addition of acetic acid. Material in the form of flock is then treated by circulation of the bath at 40° C. There are then introduced:

- 0.15 percent of 1-amino-2-bromo-N-(4-methyl-sulphophenyl)-4-amino-anthraquinone;
- 0.05 percent of [8-hydroxy-6-sulpho-2-amino-naphthalene]-<1 azo 4>-[N-phenyl-N-ethyl-2-aminosulphonyl-1-methyl-benzene]; 0.05 percent of [8-hydroxy-6-sulpho-2-amino-naphthalene]-<1 azo 4>-[2',5'-dichloro-4'-sulpho-1-phenyl-3-methyl-5-hydroxy-pyrazole].

The temperature is raised to 85° C. in a period of 40 minutes. It is maintained at this temperature for 30 minutes, and then the material is rinsed and dried.

The grey shade obtained is uniform and has a fastness equal to that which is obtained on effecting the dyeing at pH 6 and at 95° to 100° C.

I claim:

5. 1. A process for dyeing polypeptide fibers which comprises dyeing said fibers with an anionic dyestuff in the presence of (1) at least one polyoxyalkylenated non-ionic dispersing agent of the formula:



wherein  $R'$  represents an aliphatic or alkylphenyl radical containing 10 to 22 carbon atoms and  $q$  is a whole number from 10 to 50, and (2) at least one polyoxyalkylenated condensate of the formula:



wherein  $R$  represents a saturated or unsaturated aliphatic radical containing 12 to 20 carbon atoms,  $m$  and  $n$  each represents a whole number, the sum of  $m$  and  $n$  being from three to 20,  $p$  represents one or two and  $X$  represents the residue  $SO_3Y$  or the residue  $PO_3Y_2$ ,  $Y$  represents a hydrogen atom, an alkali metal, the ammonium group or the residue of an organic base of low molecular weight, wherein the ratio of the amount of non-ionic dispersing agent (1) used to the amount of polyoxyalkylenated ester (2) used is between 0.6 and 5 by weight and wherein the dyeing is effected at an approximately constant temperature not exceeding 85° C., and a pH near to the isoelectric point of the fibers.

- 25 2. A process as claimed in claim 1 wherein the fibres are first treated in an aqueous bath containing at least one anionic dispersing agent (1) and at least one polyoxyalkylenated ester (2) at a pH near to the isoelectric point of the fibres and at a temperature between 40° and 85° C., the dyestuff is then added and dyeing is effected at an approximately constant temperature not exceeding 85° C.

- 35 3. A composition comprising an aqueous mixture of (1) at least one polyoxyalkylenated non-ionic dispersing agent resulting from the condensation of an alkylene oxide with an aliphatic alcohol or an alkylphenol and (2) at least one polyoxyalkylenated condensate resulting from the condensation of an alkylene oxide with 40 an aliphatic amine containing 12 to 20 carbon atoms and esterification with an oxygen-containing polyacid.

- 45 4. A composition as claimed in claim 3 wherein the ester (2) is of the formula:



wherein  $R$  represents a saturated or unsaturated aliphatic radical containing 12 to 20 carbon atoms,  $m$  and  $n$  each represents a whole number, the sum of  $m$  and  $n$  being from three to 20,  $p$  represents one or two and  $X$  represents the residue  $SO_3Y$  or the residue  $PO_3Y_2$ ,  $Y$  representing a hydrogen atom, an alkali metal, the ammonium group or the residue of an organic base of low molecular weight.

5. A composition as claimed in claim 3 wherein the non-ionic dispersing agent (1) is of the formula:



wherein R' represents an aliphatic or alkylphenyl radical containing 10 to 22 carbon atoms and q is a whole number from 10 to 50.

6. A composition as claimed in claim 3 wherein the ratio of the amount of non-ionic dispersing agent used to the amount of polyoxyalkylenated condensate used is between 0.6 and five.

7. A composition as claimed in claim 3 wherein the polyoxylalkylenated condensate is the compound of the formula:

5



in which  $m + n = 11$  and R represents the residue of a copraamine and in which the non-ionic dispersing agent is the product resulting from the condensation of 10 11 moles of ethylene oxide with one mole of nonylphenol.

\* \* \* \* \*

15

20

25

30

35

40

45

50

55

60

65